

## UNITED STATES PATENT OFFICE

1,982,857

## HARD CEMENTED CARBIDE MATERIAL

Gregory J. Comstock, Edgewood, Pa., assignor to  
Firth-Sterling Steel Company, McKeesport, Pa.,  
a corporation of Pennsylvania

No Drawing. Application December 1, 1932,  
Serial No. 645,238

2 Claims. (Cl. 75—1)

This invention relates to hard cemented carbide materials made by a cementing or sintering process which are useful as cutting tools, wire drawing dies, and the like.

5 The composition contains a predominant proportion of titanium carbide and lesser amounts of tungsten carbide, tantalum carbide, and an auxiliary metal or metals such as cobalt, nickel and iron. The tungsten carbide is preferably present in a greater proportion than the tantalum carbide.

In my application Serial No. 641,762, filed November 8, 1932, there is disclosed a hard cemented carbide composition containing tungsten carbide, tantalum carbide, titanium carbide, and an auxiliary metal such as cobalt, nickel or iron. In that application the principal abrasive constituent is tungsten carbide, whereas in the present application the principal or predominant 20 abrasive constituent is titanium carbide.

It has been found that where a powdered mixture containing a predominant proportion of titanium carbide, and lesser amounts of tungsten carbide and tantalum carbide, and also an auxiliary metal or metals such as cobalt, nickel or iron, is sintered or cemented, a tool can be produced which has an exceptionally high capacity for cutting steel. The tool has a low heat conductivity and has a much less tendency 30 to form the detrimental chip cavity behind the cutting edge of the tool than other cemented compositions known to the prior art. It produces a smooth or plenished cut when used in the high speed machining of steel.

35 In the manufacture of the hard cemented carbide material, a powdered mixture containing a predominant proportion of titanium carbide and lesser amounts of tungsten carbide and tantalum carbide, and a metal or metals of the group consisting of cobalt, nickel and iron, is ground in a ball mill in accordance with the usual process of preparing finely divided materials for sintering. Thereafter, the powdered mixture is either first compacted and then sintered, or heat and 40 pressure may be applied simultaneously in order to produce the hard cemented carbide composition.

The proportion of titanium carbide used is 50 between about 40% and 60% by weight of the whole mixture. The tungsten carbide may be between about 20% and 40%. The tantalum carbide may vary between 5% and 20%. The cobalt, nickel or iron, or mixtures thereof, should be between 3% and 15%. The titanium carbide 55 always is present in predominating proportions.

That is, the percentage of titanium carbide is greater than any of the other carbides or the auxiliary metals. In a typical example, the mixed powders which were sintered contained,—

|                  | Percent |
|------------------|---------|
| Titanium carbide | 46      |
| Tungsten carbide | 29.62   |
| Tantalum carbide | 12.70   |
| Cobalt           | 11.68   |
|                  | 65      |

This mixture when sintered had a hardness of 79.5 Rockwell C scale and proved very efficient in the high speed machining of steel.

In making the composition, metallic tungsten may be substituted either entirely or in part for 70 the tungsten carbide. Likewise, metallic tantalum may be substituted for the tantalum carbide. Furthermore, metallic columbium or columbium carbide may be substituted for the tantalum carbide either entirely or in part. In the claims, 75 the terms "tungsten carbide" and "tantalum carbide" are intended to include the metals or carbides which I have pointed out may be substituted for the tungsten carbide and tantalum carbide. Metallic titanium or an oxide of titanium 80 such as titanium dioxide may be used to replace a small proportion, say up to 10%, of the titanium carbide. The composition may also contain, in addition to the constituents which have already been mentioned, small proportions of metallic chromium or molybdenum or their carbides. 85

For purposes of illustration, I have set forth a typical analysis of a composition embodying my invention. It is to be understood, however, that the invention may be otherwise embodied and 90 that the proportions of the constituents may vary within the scope of the following claims.

I claim:

1. A hard cemented carbide material containing about 46% titanium carbide, about 29.62% tungsten carbide, about 12.70% tantalum carbide, and about 11.68% cobalt.

2. A hard cemented carbide material consisting essentially of about 40% to 60% titanium carbide, about 20% to 40% tungsten carbide, about 5% to 20% tantalum carbide, and about 3% to 15% of a metal of the group consisting of cobalt, nickel and iron.

GREGORY J. COMSTOCK.

105

110